# EUROPEAN PATENT SPECIFICATION

(11) **EP 0 517 576 B1**
(45) Date of publication and mention of the grant of the patent: **20.03.1996**
(21) Application number: 92401496.2
(22) Date of filing: 02.06.1992
(51) Int. Cl.: C23C 8/08

(54) **Process for storing a gas mixture in passivated metal containers to enhance the stability of gaseous hydride mixtures at low concentration in contact therewith**
Verfahren zur Speicherung von Gasmischungen in passivierten Metallbehältern, um die Stabilität von gasförmigen, damit in Kontakt stehenden Hydridmischungen niedriger Konzentration zu erhöhen
Procédé pour emmagasiner un mélange gazeux dans des containers en metal passivé pour améliorer la stabilité de mélanges gazeux à faible concentration en hydrides, en contact avec ces surfaces

(30) Priority: 03.06.1991 US 709183
(43) Date of publication of application: 09.12.1992
(73) Proprietor: L'AIR LIQUIDE, SOCIETE ANONYME POUR L'ETUDE ET L'EXPLOITATION DES PROCEDES GEORGES CLAUDE, F-75321 Paris Cédex 07 (FR)
(72) Inventor: Li, Yao-En, c/o L'Air d'Orsay, F-75007 Paris (FR); Rizos, John, c/o L'Air d'Orsay, F-75007 Paris (FR); Kasper, Gerhard, c/o L'Air d'Orsay, F-75007 Paris (FR)
(74) Representative: Vesin, Jacques

(56) References cited:
- WO-A-89/12887
- GB-A- 1 530 337
- GB-A- 2 107 360
- US-A- 4 714 632

## Description

### BACKGROUND OF THE INVENTION

### Field of the Invention:

The present invention relates to a process for storing a gas mixture in passivated metal containers to enhance the stability of gaseous hydride mixtures at low concentration in contact therewith.

### Description of the Background:

In the electronics industry, and in view of environmental considerations, there is an important need for stable gas mixtures containing low concentrations of gaseous hydrides in the ppb to ppm range. The standard practice in industry is to prepare such mixtures in compressed gas cylinders, in which such mixtures are often stored for extended periods of time. However, due to reactions between gas mixtures containing such amounts of gaseous hydrides and the metal surfaces of containers containing these mixtures, it is very difficult to stabilize the same.

One approach to overcoming this instability and to maintaining a constant gas mixture concentration is to minimize the contact time between the low concentration hydrides and metal containers by storing a high concentration mixture in the cylinder and then diluting immediately before use. Unfortunately, however, in many instances, it is desirable, if not necessary, to store the gas mixtures in metal cylinders for extended periods of time.

Another approach for maintaining a constant gas mixture concentration of low concentration hydrides is saturation passivation. In this technique, the container is subjected to several cycles of evacuating and filling with a much higher concentration of the same gaseous hvdride. prior to being filled with the low concentration hydride mixture of interest. This procedure is repeated several times based upon previous empirical studies. This technique is of limited usefulness, however, as a higher concentration of the same hydride must be used for conditioning the container, and it is very disadvantageous to handle large amounts of toxic gases, such as arsine, during the process.

British Patent Specification 1530337 discloses a method to apply a protective coating to metals, particularly graphite used as a moderator in a nuclear reactor, to avoid corrosion of the same.

Thus, a need continues to exist for a passivation process which is suitable for stabilizing gaseous hydride mixtures, which avoids the drawbacks of the conventional approaches described above.

### SUMMARY OF THE INVENTION

Accordingly, it is an object of the present invention to provide a process for storing a gas mixture to enhance the stability of the gas mixture containing gaseous hydrides in low concentration in contact with a metal container.

It is also an object of this invention to provide a process for passivating a metal surface, which is advantageous for treating any metal surface, particularly those which are used to make gas storage cylinders, conduits, containers, pipes, tank truck storage rigs or railroad tank storage cars, for example.

It is, in particular, an object of the present invention to provide a process for passivating a metal surface, which is particularly advantageous for treating metal compressed gas storage cylinders.

The above objects and others which will become more apparent in view of the following are provided by a process for storing a gas mixture as defined in claim 1 to enhance the stability of a gas mixture containing gaseous hydrides in low concentration in contact therewith, which entails:
a) purging gas in contact with said metal surface with inert gas to remove the purged gas,
b) exposing the metal surface to an amount of a gaseous passivating agent comprising an effective amount of a gaseous hydride of silicon, germanium, tin or lead, and for a time sufficient to passivate said metal surface, and
c) purging the passivating agent using inert gas.

### BRIEF DESCRIPTION OF THE DRAWINGS

Figure 1 illustrates a schematic diagram of a flow system in accordance with the present invention.

Figure 2 graphically illustrates the relationship between trapping time and loss of 1 ppm ASH₃/Ar in 316 L stainless steel tubing.

### DETAILED DESCRIPTION OF THE PREFERRED EMBODIMENTS

In accordance with the present invention, a process is provided for storing a gas mixture including passivating a metal surface to enhance the stability of a gas mixture containing gaseous hydrides in low concentration in contact therewith, such as arsine, phosphine or stibine.

At present, passivation is used to improve the corrosion resistance of metal particles and steel surfaces for very particular applications. For example, WO 89/12887 describes a silane passivation process on metal particles, which improves the corrosion resistance against metallic oxidation, and GB 2,107,360 B describes a silane passivation process for steel surfaces for improving corrosion resistance in a carbon dioxide-rich environment at high temperature and pressure. However, neither of these disclose or suggest a process for stabilizing a gas mixture composition as in the present invention.

In accordance with the present process, any metal surface may be treated so as to enhance the stability of gas mixtures containing gaseous hydrides in low concentration in contact therewith. The metal surface may be, for example, metal tubing, metal valves or metal compressed gas storage cylinders. However, any type of metal surface may be so treated.

For example, in accordance with the present invention, any metal may be passivated, in particular those which are useful in making gas storage cylinders, conduits, containers, pipes and any type of storage means including railroad tank storage cars and tank truck trailer rigs. For example, metals such as iron, steel and aluminum may be passivated in accordance with the present invention.

The present invention may, for example, be advantageously used in the treatment of various steels and alloys thereof, such as ferrite steels, austenitic steels, stainless steels and other iron alloys, and is particularly advantageous in the treatment of stainless steels. However, other types of metals may be so treated.

Generally, the present invention is used to passivate a metal surface using relatively non-toxic gaseous hydrides to enhance the stability of gas mixtures containing gaseous hydrides in low concentration.

As used herein, the term "relatively non-toxic gaseous hydrides" includes the silicon hydrides, germane hydrides, tin hydrides and lead hydride. The toxic gaseous hydrides such as arsine or phosphine are avoided.

Of particular usefulness are silicon hydrides of the general formula Siₙ H₂ₙ₊₂, such as SiH₄, Si₂H₆ and Si₆H₁₄. However, other hydrides such as Ge₂H₆, Ge₉H₂₀, SnH₄, SnH₆ or PbH₄ may be used.

In the above formula for silicon hydrides, n is generally from 1 to 10. However, n can be a higher value as silicon hydrides are known to exhibit catenation. See Advanced Inorganic Chemistry, Cotton and Wilkinson, Third Edition.

As used herein, the phrase "gaseous hydrides in low concentration" generally means gaseous hydrides of a concentration of from about 10 ppb to about 10 ppm. More preferably, the concentration is about 50 ppb to about 5 ppm. Most preferably, however, the concentration about 100 ppb to about 1 ppm.

In accordance with the present invention in order to passivate a metal surface to enhance the stability of a gas mixture containing gaseous hydrides in low concentration in contact therewith, it is first necessary to purge the gas or gas mixture initially in contact with the metal surface with inert gas to remove the purged gas. As an inert purging gas, any gas which is generally chemically non-reactive may be used. For example, the so-called noble gases, such as krypton, xenon, helium, neon and argon may be used. However, other gases such as hydrogen and nitrogen may be used. Generally, the inert purging gas will be passed over the metal surface for a time and in an amount sufficient to remove substantially all of the purged gas. Typically, the purging gas is passed over the metal surface, or through a volume defined by a continuous metal surface, such as a compressed gas storage cylinder, for anywhere from several seconds to up to about 30 minutes at from 101 325 Pascal (1 atm.) to about 303975 Pascal (3 atm.) of pressure. However, higher Dressures may be used, if desired.

In accordance with the present invention, nitrogen has been found to be advantageous as an inert purging gas, although other inert aases may be used.

After purging the gas in contact with the metal surface, the metal surface is then exposed to an amount of passivating agent containing an effective amount of one or more gaseous hydrides of silicon, germanium, tin or lead, and for a time sufficient to passivate the metal surface.

Generally, the higher the concentration of passivating agent used, such as silane, the shorter the exposure time required. However, passivating agent concentrations of as low as 1 ppm may be used, or as high as 100%. For example, if a very low concentration of silane is used, exposure times in excess of 80 hours are usually required. Generally, exposure times of about 100 hours are typically used for dilute passivating agents. However, if relatively pure passivating agent is used, for example, generally less than 60 minutes exposure time is required, preferably less than 30 minutes.

As described above, the phrase "pure passivating agent" means that the passivating agent used is the pure gaseous hydride of one or more silicon, germanium, tin or lead.

While any concentration of passivating agent may be used, it is generally desirable to use a concentration in the range of about 0.01% to 20% by volume. It is preferred, however, to use a concentration in the range of about 0.01% to 5% by volume. With such concentrations, an exposure time of from about 1 to 24 hours is generally required. Generally, for larger metal surfaces, such as vessels, larger volumes of passivating agent may be used.

In accordance with the present invention, substantially all of the purged gas is displaced or removed by the inert gas.

As used herein, the phrase "substantially all of the purged gas" means that the purged gas is removed to an extent of above 99% by volume.

Generally, the purged gas is air, however, other gases or gas mixtures, such as mixtures mainly containing nitrogen and oxygen, may be purged in accordance with the present invention.

Generally, the exposure of the metal surface to the passivating agent may be effected at from very low temperatures of about -20°C to up to right below the gaseous hydride decomposition temperature of the one or more gaseous hydrides in the passivating agent. For example, the decomposition temperature of silane is 250°C. However, it is generally preferable to effect the exposure at from about 10°C to about 100°C. It is more preferable to effect the passivating agent exposure at from about 20°C to about 50°C. However, it is most advantageous to effect the exposure at about 25°C.

Although the exposure may be effected at high temperatures, the gas phase reaction of the one or more gaseous hydride of the passivating agent, such as silane, is preferably kept to a minimum to avoid the formation of particles. Generally, this means at a temperature of less than the passivating agent gaseous hydride decomposition temperature.

After subjecting the metal surface to treatment with passivating agent, the latter is, itself, purged with an inert purging gas, such as nitrogen. However, the noble gases as described above may be used.

The present invention also provides an optional fourth step in which the metal surface is then exposed to an oxidizing gas in order to stabilize the adsorbed passivating agent on the metal surface. As an oxidizing gas, gas mixtures containing nitrogen and oxygen may be used, for example.

Generally, oxidizing gas mixtures may be used which are capable of oxidizing the adsorbed passivating agents to an inert oxidized form. For example, gas mixtures containing from about 1 to 10% volume of oxygen in nitrogen may be advantageously used when using such mixtures to oxidize the adsorbed passivating agent, metal surface exposure times of film about 30 sec. to about 3 minutes are generally used. However, shorter or longer exposure times may be used as required.

In general, the oxidation step may be effected at the same temperatures as used for the passivation step, with temperatures of from about 10°C to about 100°C being preferred, and with temperatures of from 20°C to about 50°C being most preferred.

In accordance with this aspect of the present invention it has been discovered that adsorbed gaseous hydride may be desorbed very slowly over a period of time thus reducing the effectiveness of the passivation treatment over time. By oxidizing the adsorbed passivating agent containing a gaseous hydride, such as silane, for example, an inert compound, such as SiO₂, may be formed. Hence, the oxidation step provides a means to stabilize the passivated metal surface for long term use.

Figures 1 and 2 will now be described in more detail.

Figure 1 provides a schematic flow diagram using mass flow controllers, an arsine permeation device, valves and port valves A and B in fluid connection. This apparatus is conveniently used to test the stability of gaseous hydrides, as measured by an inductively coupled plasma spectrophotometer. However, other detection means known to those skilled in the art may be used instead.

Figure 2 illustrates a summary of stability data from samples A, B and C as defined hereinbelow in the example. In particular, the 1 ppm treatment (sample C) failed to passivate the metal surface after 69 hours of exposure. Generally, at such low concentrations, in excess of 70 hours of exposure is required, preferably at least 80 hours of exposure.

The pure silane treatment (sample B) effected surface passivation in less than 30 minutes of exposure. Sample A is a controlled sample.

Generally, in accordance with the present invention, the gaseous hydride treatment is effected to passivate substantially all of the metal surface. As used herein, the term "substantially all" means that at least 90% of the metal surface in contact with the gaseous hydride is passivated. However, it is preferred if at least 99% of the metal surface in contact with the gaseous hydride is passivated. It is particularly preferred if at least 99.9% of the metal surface in contact with the gaseous hydride is passivated.

The present invention will now be further illustrated by reference to certain examples which are provided for purposes of illustration and are not intended to be limitative.

### Example

In order to demonstrate the effect of the present invention on metal surfaces, a 0.635 cm (1/4") ID stainless steel tube was used.

Three identical samples (A, B and c) of 1/4" ID stainless steel tubings were exposed to ambient air under the conditions typical in the preparation of gas handling and storage equipment. It is known that under such exposure conditions, the stability of mixtures is very poor. All of the samples were then purged with dry N₂ gas at room temperature. Sample A served as a controlled sample. Sample B was then treated with flowing pure silane for 30 minutes at room temperature and sample C was purged with 1 ppm silane for 72 hours, followed by purging with dry air, according to the conditions described below.

The stability of hydrides in the so prepared samples A, B and C was tested in a setup as shown in Figure 1. The tube was filled with argon gas containing 1 ppm arsine. This gas was kept in the tube by means of the valve 2 in Figure 1 for various periods of time. After that, the gas was introduced into a device capable of measuring the concentration of hydride remaining in the gas. In this example, the device is an Inductively coupled plasma spectrophotometer. However, other detection means may be used. The ratio of initial fill concentration to final concentration was used to measure the gas stability. The results for a typical test with arsine are shown in Figure 2.

Additionally, the present Invention also provides storage means for a gas or gas mixture, which means at least has an interior metal surface thereof which has been passivated. However, the storage means may be completely made of metal. Preferabty, the storage means is compressed gas storage cylinder. However, the storage means may be a mobile storage means, such as a tank tractor trailer rig or a railroad tank car.

Thus, the present invention provides storage means having at least an interior metal surface thereof which is passivated, thereby enhancing the stability of a gas mixture containing one or more gaseous hydrides in low concentration when in contact therewith. As used herein, the term "passivated" means that the internal metal surface of the storage means has been subjected to the present passivation process and is thus unable to react with gases or gas mixtures stored therein which contain low concentrations of gaseous hydrides. In accordance with the present invention, it is advantageous if the passivating agent used is a silicon hydride of the formula Siₙ H₂ₙ₊₂, wherein n is 1-10, more preferably n is 1.

It is, however, particularly preferred if the passivated storage cylinder whose internal surface has been passivated with gaseous hydride passivating agent in accordance with the present process.

## Claims

1. A process for storing a gas mixture in a container or the like, said gas mixture containing one or more gaseous hydrides in a concentration from about 10ppb to about 10ppm, which comprises:
a) providing a container or the like having an internal metal surface,
b) purging gas in contact with said metal surface with inert gas to remove said purged gas,
c) exposing the metal surface to an amount of a passivating agent comprising an effective amount of gaseous hydride of silicon, germanium, tin or lead, and for a time sufficient to passivate said metal surface,
d) purging said passivating agent using inert gas, and
e) storing said gas mixture in said container or the like; thereby enhancing the stability of said gas mixture.

2. The process according to Claim 1, wherein said metal surface comprises steel, iron or aluminum.

3. The process according to Claim 1 or 2, wherein said container is a compressed gas storage cylinder, a tank tractor trailer rig, a railroad rank car, a container, a conduit and/or a pipe.

4. The process according to one of Claims 1 to 3, wherein said purged gas is air.

5. The process according to one of Claims 1 to 4, wherein said inert gas is nitrogen, argon, krypton, xenon or neon.

6. The process according to one of Claims 1 to 5, which further comprises, after step d), exposing the metal surface to an oxidizing gas or gas mixture in an amount and for a time sufficient to stabilize the adsorbed passivating agent on the metal surface.

7. The process according to one of Claims 1 to 6, wherein said one or more gaseous hydrides in low concentration are selected from the group consisting of phosphine, arsine and stibine.

8. The process according to one of Claims 1 to 7, wherein said gaseous hydride passivating agent is selected from the group consisting of a silicon hydride of the formula Siₙ H₂ₙ₊₂, wherein n is 1 to 10; Ge₂H₆, Ge₉H₂₀, SnH₄, SnH₆ and PbH₄.

9. The process of Claim 8, wherein said gaseous hydride passivating agent is a silicon hydride of the formula SiₙH₂ₙ₊₂, wherein n is from 1 to 10.

10. The process of Claim 9, wherein said silicon hydride is SiH₄.

## Patentansprüche

1. Verfahren zur Speicherung eines Gasgemischs in einem Behälter oder ähnlichem, wobei das Gasgemisch ein oder mehrere gasförmige Hydride in einer Konzentration von etwa 10ppb bis etwa 10ppm umfaßt, mit folgenden Schritten:
a) zur Verfügung stellen eines Behälters oder ähnlichem mit einer inneren metallischen Oberfläche,
b) Abreinigen von Gas, welches sich in Kontakt mit der Metalloberfläche befindet, mittels eines Edelgases, um das abgereinigte Gas zu entfernen,
c) in Kontakt bringen der Metalloberfläche mit einer Menge eines Passivierungsmittels, welches eine wirksame Menge an gasförmigem Hydrid von Silizium, Germanium, Zinn oder Blei enthält während einer Zeitspanne, die ausreicht, um die Metalloberfläche zu passivieren,
d) Abreinigen des Passivierungsmittels mittels Edelgas, und
e) Speichern des Gasgemisches in dem Behälter oder ähnlichem; wodurch die Stabilität des Gasgemisches erhöht wird.

2. Verfahren nach Anspruch 1, wobei die Metalloberfläche Stahl, Eisen oder Aluminium umfaßt.

3. Verfahren nach Anspruch 1 oder 2, wobei der Behälter ein Druckgas-Speicherzylinder, eine Tanklastzug-Anhänger-Garnitur, ein Eisenbahntankwagen, ein Behälter, eine Leitung und/oder ein Rohr ist.

4. Verfahren nach einem der Ansprüche 1 bis 3, wobei das abgereinigte Gas Luft ist.

5. Verfahren nach einem der Ansprüche 1 bis 4, wobei das Edelgas Stickstoff, Argon, Krypton, Xenon oder Neon ist.

6. Verfahren nach einem der Ansprüche 1 bis 5, wobei nach Schritt d) die Metalloberfläche mit einem oxidierenden Gas oder einem Gasgemisch in Kontakt gebracht wird, und zwar in einer Menge und während einer Zeitspanne, die ausreicht, um das adsorbierte Passivierungsmittel auf der Metalloberfläche zu stabilisieren.

7. Verfahren nach einem der Ansprüche 1 bis 6, wobei ein oder mehrere gasförmige Hydride in niedriger Konzentration aus der Phosphin, Arsin und Stibin umfassenden Gruppe ausgewählt sind.

8. Verfahren nach einem der Ansprüche 1 bis 7, wobei das gasförmige Hydrid-Passivierungsmittel aus der Gruppe ausgewählt ist, die Siliziumhydrid der Formel Siₙ H₂ₙ₊₂ (n gleich 1 bis 10), Ge₂H₆, Ge₉H₂₀, SnH₄, SnH₆ und PbH₄ umfaßt.

9. Verfahren nach Anspruch 8, wobei das gasförmige Hydrid-Passivierungsmittel ein Siliziumhydrid der Formel SiₙH₂ₙ₊₂ ist, wobei n gleich 1 bis 10 ist.

10. Verfahren nach Anspruch 9, wobei das Siliziumhydrid SiH4 ist.

## Revendications

1. Procédé de stockage d'un mélange gazeux dans un réservoir ou un élément similaire, ledit mélange gazeux contenant un ou plusieurs hydrures gazeux dans une concentration allant d'environ 10 ppb à environ 10 ppm, qui comprend:
a) la mise à disposition d'un réservoir ou d'un élément similaire ayant une surface métallique interne,
b) la purge du gaz en contact avec ladite surface métallique à l'aide d'un gaz inerte afin d'éliminer ledit gaz purgé,
c) l'exposition de la surface métallique à une quantité d'un agent de passivation comprenant une quantité efficace d'hydrure gazeux de silicium, de germanium, d'étain ou de plomb, et pendant une période suffisante à passiver ladite surface métallique,
d) la purge dudit agent de passivation en utilisant un gaz inerte, et
e) le stockage dudit mélange gazeux dans ledit réservoir ou dans un élément similaire; améliorant ainsi la stabilité dudit mélange gazeux.

2. Procédé selon la revendication 1, caractérisé en ce que ladite surface métallique comprend de l'acier, du fer ou de l'aluminium.

3. Procédé selon la revendication 1 ou 2, caractérisé en ce que ledit réservoir est un cylindre de stockage de gaz comprimé, un ensemble semi-remorque tracté de camion-citerne, un wagon-citerne ferroviaire, un réservoir, un conduit et/ou une canalisation.

4. Procédé selon l'une quelconque des revendications 1 à 3, caractérisé en ce que ledit gaz purgé est l'air.

5. Procédé selon l'une quelconque des revendications 1 à 4, caractérisé en ce que ledit gaz inerte est l'azote, l'argon, le krypton, le xénon ou le néon.

6. Procédé selon l'une quelconque des revendications 1 à 5, qui comprend en outre, après l'étape d), l'exposition de la surface métallique à un gaz ou un mélange gazeux oxydant dans une quantité et une période de temps suffisantes pour stabiliser l'agent de passivation adsorbé sur la surface métallique.

7. Procédé selon l'une quelconque des revendications 1 à 6, caractérisé en ce que ledit hydrure gazeux ou lesdits hydrures gazeux à basse concentration est choisi ou sont choisis parmi le groupe se composant des phosphines, des arsines et des stibines.

8. Procédé selon l'une quelconque des revendications 1 à 7, caractérisé en ce que ledit agent de passivation d'hydrure gazeux est choisi parmi le groupe se composant d'un hydrure de silicium de formule SiₙH₂ₙ₊₂, dans laquelle n va de 1 à 10; Ge₂H₆, Ge₉H₂₀, SnH₄, SnH₆ et PbH₄.

9. Procédé de la revendication 8, caractérisé en ce que ledit agent de passivation d'hydrure gazeux est un hydrure de silicium de formule SiₙH₂ₙ₊₂, dans laquelle n va de 1 à 10.

10. Procédé de la revendication 9, caractérisé en ce que ledit hydrure de silicium est SiH₄.
